

## UNITED STATES PATENT OFFICE

2,516,139

METHOD OF AND MATERIAL FOR TREATING  
FERRIFEROUS METAL SURFACES WITH  
MANGANESE PHOSPHATE COATING SO-  
LUTIONSJoseph Mazia, Philadelphia, Pa., assignor to  
American Chemical Paint Company, Ambler,  
Pa., a corporation of DelawareNo Drawing. Application December 8, 1948,  
Serial No. 64,247

7 Claims. (Cl. 148—6.15)

1

This invention relates to the phosphate coating art and particularly to that art as applied to the treatment of ferriferous surfaces where a manganese phosphate coating solution is employed. Of course, the basic principles of phosphate coating are well known to those skilled in the art so the present disclosure will refer only briefly to the technique employed. Suffice it to say that it has long been the practice to prepare and maintain the coating bath or solution in a saturated or substantially saturated condition with respect to the metallic phosphate in equilibrium with the liquid and that the solution may be applied to the surface which is to be treated in any one of a number of ways, i. e., by dipping the work into the solution or by flowing or spraying the solution over the surface. This requires that the coating bath or solution contain a certain minimum quantity of free acid. If the acidity be reduced, the solution becomes so supersaturated with respect to the metallic phosphate that some of the phosphate is precipitated as a solid phase. This precipitation (actually a mere crystallization of a constituent from a supersaturated solution) is commonly known as "sludging out." Heretofore such "sludging out" has constituted a major problem to the users of these processes and materials and the present invention is particularly directed toward a solution of this problem.

The principal objects of the present invention are to provide a method of as well as a material for use in the treatment of ferriferous metals with manganese phosphate coating solutions whereby so-called "sludging out" is substantially eliminated or at least so greatly minimized or inhibited as to render the problem of disposing of the sludge of no serious consequence. Another object is to provide a manganese phosphate coating solution which has a much greater degree of stability than coating solutions now commonly in use, as well as to provide a composition or material from which the bath or solution may be prepared or maintained in proper working condition. Another object is to provide a concentrated composition or material which can be utilized by simple dilution with water. Still another object is to provide a method of and material for use in manganese phosphate coating operations by means of which

2

any substantial incrustation or build-up of deposit on the heating surfaces is avoided or at least greatly minimized which, of course, makes it easier to maintain a uniform bath temperature and aids in reducing maintenance costs.

Before proceeding with a detailed description of the present invention I wish to define "stability" as employed herein. This refers to the degree to which an acid phosphate solution of 10 the character described resists spontaneous disturbance of its state of acidity, (or its pH). As is well known in this art, where supersaturated acid phosphate coating solutions are employed, there is a tendency for the solutions to increase 15 in acidity. Therefore, increase in acidity accompanies a loss in supersaturation and the loss in supersaturation is evidenced by the "sludging out" already referred to. This, of course, is accompanied by a decrease in the pH of the solution.

The present invention is based upon the discovery that the addition of certain tartrate ions to an otherwise conventionally formulated manganese phosphate coating bath imparts to the bath a very great degree of stability and makes it possible to operate such baths in a relatively 25 sludge free condition for long periods of time. This, of course, results in a much more economical process because the bath does not lose excessive quantities of the actual coating-producing ingredients in the sludge forming phenomenon.

With the exception of the ions of meso tartaric acid the tartrate ions may be introduced in any form desired as long as due regard to solubility 35 and chemical compatibility of the compound are considered. For example, they may be introduced as potassium acid tartrate (cream of tartar). I prefer to use cream of tartar inasmuch as the addition of this material has little effect on the pH of the ordinary coating bath. If tartaric acid is used as a source of the tartrate ion, then enough neutralizing material 40 such as caustic alkali, manganese carbonate, etc., must be added to the bath to adjust the pH of the bath to bring it back within proper operating coating range. Contrariwise, if Rochelle salts are used, a suitable acid such as phosphoric acid 45 must be added to the bath to adjust the starting pH. Such adjustments in the degree of acidity

are expedients familiar to those skilled in the art of phosphate coating.

In order to bring out more fully the nature of the present invention, the following illustrative examples are given. For instance a concentrated composition may be prepared as follows:

*Formula I*

|                                        |        |     |
|----------------------------------------|--------|-----|
| Manganese carbonate, 85%               | grams  | 200 |
| Phosphoric acid, 75%                   | do     | 550 |
| Cream of tartar (potassium bitartrate) | do     | 20  |
| Water, to make                         | liters | 1   |

The foregoing formula produces a concentrated material which can be prepared for use by simple dilution with water and it will be noticed that the ratio of tartrate ion, calculated as tartaric acid, to manganese equals 0.196. In preparing a working bath or solution 10% by volume of the foregoing concentrate is employed. Such a bath shows no "sludging out" even at the boiling point and produces excellent coatings on ferriferous metal surfaces. If the bath be prepared from the same concentrate minus only the cream of tartar, a very definite "cloud point" is reached at about 150° F., the "cloud point" being the point where "sludging out" becomes evident. At higher temperatures sludge formation becomes heavy.

*Formula II*

|                                |        |      |
|--------------------------------|--------|------|
| Manganese carbonate, 85%       | grams  | 193  |
| Phosphoric acid, 75%           | do     | 546  |
| Sodium nitrate                 | do     | 61   |
| Sodium bitartrate, monohydrate | do     | 18.5 |
| Water, to make                 | liters | 1    |

The foregoing formula yields another concentrated composition or material which, as before, can be diluted with water in the ratio of 10% by volume of solution. The ratio of tartrate ion, calculated as tartaric acid, to manganese equals 0.186. The sodium nitrate is an expediting agent familiar to those skilled in the art.

Excellent coatings were produced by this bath with substantially no sludge formation even at the boiling point, whereas, the same bath, when prepared from a concentrate containing no sodium bitartrate, developed a "cloud point" at approximately 150° F. with heavy sludge formation at higher temperatures.

Another concentrated formula which gives excellent results is the following:

*Formula III*

|                          |         |        |
|--------------------------|---------|--------|
| Manganese carbonate, 85% | pounds  | 1.6225 |
| Phosphoric acid, 75%     | gallons | 0.3489 |
| Potassium permanganate   | pounds  | 0.0003 |
| Iron filings             | do      | 0.0406 |
| Potassium bitartrate     | do      | 0.2080 |
| Water, to make           | gallons | 1      |

This yields a ratio of tartrate ion, calculated as tartaric acid, to manganese of 0.2525 and a bath containing 10% by volume in water may be prepared and heated gradually to an operating temperature of approximately 205° F. It is then "broken in" in the normal fashion familiar in this art by allowing it to act on metallic iron. This bath will produce heavy corrosion retardant phosphate coatings in customary periods of treatment, which coatings are useful also as anti-friction surfaces of the nature familiar to those skilled in this art. The bath functions practically without sludging, whereas an identical bath with-

out the tartrate will form copious quantities of sludge during heating and breaking in as well as in regular service.

The potassium permanganate and the iron filings of the above formula are introduced for reasons familiar to those skilled in this art. For instance, the potassium permanganate will oxidize a portion of the ferrous iron to yield a small quantity of the substantially insoluble ferric phosphate which latter tends to inhibit hydrolysis in accordance with the teachings of U. S. Patent 2,316,810. The iron filings also aid in the breaking in of the solution. However, I wish it to be distinctly understood that neither of these materials is in any way essential to a realization of invention.

In all of the foregoing formulas the preferable operating temperature is under the boiling point and preferably in the neighborhood of 205° F. as just indicated in connection with Formula III.

It will be noted from the foregoing that relatively very small amounts of tartrate ion in the bath have a stabilizing effect, but I have found that the beneficial effects of my invention can be secured within a rather wide range of tartrate ion. Experience has shown that best results are secured by operating with baths which contain from 0.5 gram per liter to approximately 15 grams per liter of the tartrate ion expressed as dextro tartaric acid. Below a concentration of 0.5 gram per liter the tartrate ion has a reduced stabilizing effect and as the concentration nears 15 grams per liter the coatings, on certain types of surfaces, may exhibit a lack of continuity, and when the tartrate ion exceeds 15 grams per liter, the phosphate coating may have a white precipitate formed thereon, which, for some uses, may be objectionable.

Expressed in terms of the relationship between the tartrate ion and the manganese, I have found that the ratio of tartrate ion (calculated as dextro tartaric acid) to manganese should lie between approximately 0.03 and 1.5.

In conclusion I should like to point out that it is well known in this art that the lower the temperature of the manganese phosphate coating bath, other things being equal, the higher must be the pH. At any given temperature there exists a pH corresponding to the equilibrium of the solution with the particular solid phosphate. At a higher pH the solution is supersaturated and tends to form "sludge" with the liberation of acid in the solution. Operating baths at or above the pH of equilibrium is common practice in this art. In any case, the action of the solution on the metal to be coated consumes acid and raises the pH in the neighborhood of the metal. This action is quite normal and necessary to cause the deposition of the desired coating. Usually, however, in the practice of the prior art, not all the solid phosphate deposited remains upon the metal surface as a coating. Some remains loose in the solution and forms a sludge. However, by using tartrate ion in accordance with my invention it is possible to operate at a higher pH than it otherwise would be without an increase in the formation of sludge which, of course, may be a distinct advantage in certain situations. For instance, by operating at a higher pH, it is sometimes possible to lower the operating temperature of the bath.

Finally, I again want to emphasize the fact that my experimental work has shown that tartrate ions from dextro and levo tartaric acid as well as from dextro-levo (racemic) acid will func-

tion satisfactorily in accordance with the teachings of this invention, whereas, ions from meso tartaric acid will not so function. Just why this is, I do not know, but in the following claims I have excluded the ions of meso tartaric acid. Broadly speaking ions from the other acids may be used in whatever quantity is necessary to have a stabilizing effect sufficient to be of value in this art and they can be used in any manganese phosphate coating bath consisting of coating-producing proportions of the ions of phosphoric acid and of manganese.

I claim:

1. In the art of treating ferriferous metal surfaces with a manganese phosphate coating bath, the method which consists in preparing an acid manganese phosphate bath containing the ions of a tartaric acid other than mesotartaric acid in quantity sufficient to substantially inhibit "sludging out" of metallic phosphate, and treating the surface with the bath to form the desired coating.

2. The method of claim 1 in which the bath contains from 0.5 to 15 grams per liter of tartrate ions calculated as tartaric acid.

3. A substantially supersaturated acid manganese phosphate coating bath containing from 0.5 to 15 grams per liter of tartrate ions other than the ions of mesotartaric acid calculated as tartaric acid.

4. In the art of treating ferriferous metal surfaces with an acid manganese phosphate coating bath, a composition for preparing or replenishing the coating bath consisting essentially of materials capable of yielding manganese ions and phosphate ions and a compound capable of yielding tartrate ions other than those of mesotartaric acid, the amount of said compound being sufficient to yield in the finished bath enough of

said tartrate ions to substantially inhibit the formation of sludge.

5. In the art of treating ferriferous metal surfaces with an acid manganese phosphate coating bath, a composition for preparing or replenishing the bath upon mixture with water, said composition consisting essentially of ingredients capable of yielding, in the bath, the desired coating-producing proportions of the ions of phosphoric acid and manganese together with a material yielding tartrate ions other than the ions of mesotartaric acid, in a ratio of tartrate ion (calculated as tartaric acid) to manganese of from 0.03 to 1.5.

15 6. In the art of treating ferriferous metal surfaces with an acid manganese phosphate coating bath, a concentrated, water-dilutable solution consisting essentially of manganese phosphate coating ingredients capable of yielding, in the bath, the desired coating-producing proportions of the ions of phosphoric acid and manganese together with a compound capable of yielding tartrate ions other than those of mesotartaric acid in a ratio of tartrate ion (calculated as tartaric acid) to manganese of from 0.03 to 1.5.

20 7. A manganese phosphate coating bath consisting essentially of an acid manganese phosphate solution containing from 0.5 to 15 grams per liter of tartrate ions other than the ions of mesotartaric acid, calculated as tartaric acid.

JOSEPH MAZIA.

#### REFERENCES CITED

The following references are of record in the 35 file of this patent:

#### UNITED STATES PATENTS

| Number    | Name             | Date         |
|-----------|------------------|--------------|
| 2,331,196 | Jernstedt et al. | Oct. 5, 1943 |